



US005516381A

# United States Patent [19]

Kawai et al.

[11] Patent Number: 5,516,381

[45] Date of Patent: \*May 14, 1996

[54] ROTATING BLADE OR STATIONARY VANE  
OF A GAS TURBINE

[75] Inventors: Hisataka Kawai; Ikuo Okada; Ichiro  
Tsugi; Koji Takahashi, all of Takasago;  
Kensho Sahira; Akira Mitsuhashi,  
both of Omiya, all of Japan

[73] Assignees: Mitsubishi Materials Corporation;  
Mitsubishi Jukogyo Kabushiki  
Kaisha, Tokyo, Japan

[\*] Notice: The term of this patent shall not extend  
beyond the expiration date of Pat. No.  
5,431,750.

[21] Appl. No.: 377,925

[22] Filed: Jan. 25, 1995

## Related U.S. Application Data

[62] Division of Ser. No. 901,241, Jun. 19, 1992, Pat. No.  
5,431,750.

## Foreign Application Priority Data

Jun. 27, 1991 [JP] Japan 3-183056

[51] Int. Cl. 6 C22C 19/05

[52] U.S. Cl. 148/410; 420/443; 420/444;  
420/448; 416/241 R

[58] Field of Search 420/443, 444,  
420/448; 416/241 R; 148/410

## [56] References Cited

### U.S. PATENT DOCUMENTS

|           |         |               |         |
|-----------|---------|---------------|---------|
| 3,459,545 | 8/1969  | Bieber et al. | 420/448 |
| 3,765,879 | 10/1973 | Hockin et al. | 420/448 |
| 4,719,080 | 1/1988  | Duhl et al.   | 420/443 |
| 5,055,147 | 10/1991 | Henry         | 420/443 |
| 5,077,141 | 12/1991 | Naik et al.   | 428/680 |

### FOREIGN PATENT DOCUMENTS

|         |         |                    |   |
|---------|---------|--------------------|---|
| 705385  | 3/1965  | Canada             | . |
| 0361084 | 4/1990  | European Pat. Off. | . |
| 0381828 | 8/1990  | European Pat. Off. | . |
| 0413439 | 2/1991  | European Pat. Off. | . |
| 220845  | 4/1985  | German Dem. Rep.   | . |
| 1-59344 | 12/1989 | Japan              | . |
| 1511562 | 5/1978  | United Kingdom     | . |

Primary Examiner—George Wyszomierski

Attorney, Agent, or Firm—Frishauf, Holtz, Goodman,  
Langer & Chick

## [57] ABSTRACT

A rotating blade or stationary vane of a gas turbine which is made of a nickel alloy containing Cr, Co, Mo, W, Ta, Al, Ti, C, B, Zr, and one or both of Mg and Ca. Additionally, the alloy may contain Hf, Pt, Rh and Re.

15 Claims, No Drawings

## ROTATING BLADE OR STATIONARY VANE OF A GAS TURBINE

This is a division of application Ser. No. 07/901,241 filed Jun. 19, 1992 now U.S. Pat. No. 5,431,750.

### BACKGROUND OF THE INVENTION

This invention relates to castable Ni-base heat-resistant alloys suitable for use as materials that form the rotating blades and stationary vanes of a gas turbine, and other machine parts that are to be subjected to elevated temperatures.

Nickel-base heat-resistant alloys that are predominantly used as constituent materials for producing the rotating blades and stationary vanes of a gas turbine, the moving vanes of a hot blower and other machine parts that are to be subjected to elevated temperatures are those which are both precipitation hardened with the  $\gamma'$  phase  $\{Ni_3(Al, Ti)\}$  and solid-solution hardened with Mo, W, etc. See, for example, Japanese Patent Publication No. 59344/1989 which describes a Ni-base heat-resistant alloy that has high strength and high resistance to oxidation and corrosion at elevated temperatures and which consists, by weight percent (all percentages that follow are on a weight basis), of 7-13% Cr, no more than 35% Co, no more than 8% Mo, no more than 3% Nb, no more than 14% W, no more than 6% Ta, 4-7% Al, 0.5-6% Ti (provided  $Al+Ti=6.5-10.5\%$ ), no more than 1.5% V, no more than 0.2% Zr, 0.7-5% Hf, 0.02-0.5% C and 0.002-0.2% B, with the remainder being Ni and incidental impurities. If the addition of Mo, W, etc. to those alloys is excessive, deleterious phases such as the  $\alpha$  and  $\mu$  phases will develop and, hence, Al and Ti are added in large amounts so that more of the  $\gamma'$  phase will develop to give higher strength at elevated temperatures.

In such predominant Ni-base heat-resistant alloys, Mo and W are added in large amounts to an extent that will not cause the formation of any deleterious phases in the alloy structure and this inevitably limits the Cr content to 7-13%. Under the circumstances, the high-temperature strength of the alloys is improved but, on the other hand, their resistance to oxidation and corrosion at elevated temperatures is so much reduced that the alloys can only be used as constituent materials for fabricating gas turbines of a type that operates on high-grade fuels which emit smaller amounts of oxidizing and corrosive materials upon combustion. It has therefore been required to develop Ni-base heat-resistant alloys that can be used as constituent materials for fabricating gas turbines of a type that can produce a higher output power even if they are operated on low-grade fuels.

### SUMMARY OF THE INVENTION

The present inventors conducted intensive studies in order to meet that requirement and, as a result, they found that the high-temperature strength of Ni-base heat-resistant alloys could be improved without compromising their resistance to oxidation and corrosion at elevated temperatures when the Cr content was adjusted to a slightly higher level of 13.1-15% with W, Mo, Al, Ti, Ta, C, B, Zr and other elements being added in such amounts as to attain the best possible balance and when the adverse effects of impurities such as oxygen and sulfur were suppressed by adding Mg and/or Ca in a total amount of 1-100 ppm. It was also found that Ni-base alloys with such balanced properties could be used as a constituent material for fabricating not only gas turbines that operate on high-grade fuels but also those

which operate on low-grade fuels such as heavy oils. The present invention has been accomplished on the basis of these findings.

The Ni-base heat-resistant alloy of the present invention has high strength and high resistance to oxidation and corrosion at elevated temperatures and consists of 13.1-15.0% Cr, 8.5-10.5% Co, 1.0-3.5% Mo, 3.5-4.5% W, 3.0-5.5% Ta, 3.5-4.5% Al, 2.2-3.2% Ti, 0.06-0.12% C, 0.005-0.025% B, 0.010-0.050% Zr and 1-100 ppm of Mg and/or Ca, in the optional presence of 0-1.5% Hf and/or 0-0.5% of at least one element selected from among Pt, Rh and Re, with the remainder being Ni and incidental impurities.

### DETAILED DESCRIPTION OF THE INVENTION

The criticality of the respective elements to be contained in the Ni-base heat-resistant alloy of the present invention is described below.

Cr: 13.1-15.0%

Gas turbines for industrial applications are required to have high resistance to oxidation and corrosion at elevated temperatures since they are exposed during operation to combustion gases that contain oxidizing and corrosive materials. Chromium is an element that imparts oxidation and corrosion resistance to the alloy of the present invention and its effectiveness becomes more significant as its content in the alloy increases. If the Cr content is less than 13.1%, it will not exhibit its intended effect. On the other hand, the Ni-base alloy of the present invention also contains Co, Mo, W, Ta, etc., so in order to attain balance with these elements, Cr should not be added in amounts exceeding 15%. Hence, the Cr content of the Ni-base alloy of the present invention is specified to lie within the range of 13.1-15.0%, preferably 13.7-14.3%.

Co: 8.5-10.5%

With Ni-base alloys of a type that can be hardened by precipitation of the  $\gamma'$  phase due to the addition of Ti and Al, the mentioned elements are thoroughly dissolved in the matrix by a solid-solution treatment and, in the subsequent aging treatment, those elements are precipitated uniformly and finely, thereby forming the  $\gamma'$  phase which contributes better strength at elevated temperature.

Cobalt is effective in improving the strength of the Ni-base alloy by enhancing the solubility limit, or the limit to which Ti and Al exhibiting the effects described above can be dissolved in the matrix at elevated temperatures. Assuming the Al and Ti contents specified for the alloy of the present invention, Co must be present in an amount of at least 8.5%. If the Co content exceeds 10.5%, the balance with other elements such as Cr, Mo, W, Ta, Al and Ti is upset, causing lower ductility due to the precipitation of deleterious phases. Hence, the Co content of the Ni-base alloy of the present invention is specified to lie within the range of 8.5-10.5%, preferably 9.5-10.5%.

Ti: 2.2-3.2%

Titanium is the element necessary for precipitation of the  $\gamma'$  phase in order to enhance the high-temperature strength of the precipitation-hardenable Ni-base alloy of the present invention. If the Ti content is less than 2.2%, the precipitation hardening by the  $\gamma'$  phase is insufficient to attain the required strength. If the Ti content exceeds 3.2%, precipitation of the  $\gamma'$  phase is so substantial as to impair the ductility of the alloy. Hence, the Ti content of the Ni-base alloy of the present invention is specified to lie within the range of 2.2-3.2%, preferably 2.5-2.9%.

Al: 3.5–4.5%

Aluminum is an element that exhibits the same effect as Ti; it contributes to the formation of the  $\gamma$  phase, thereby enhancing the high-temperature strength of the alloy. In addition, Al helps impart oxidation and corrosion resistance to the alloy at elevated temperatures. For achieving the intended effects, Al must be contained in an amount of at least 3.5%. If the Al content exceeds 4.5%, the ductility of the alloy is impaired. Hence, the Al content of the Ni-base alloy of the present invention is specified to lie within the range of 3.5–4.5%, preferably 3.8–4.2%.

Mo: 1.0–3.5%

Molybdenum will dissolve in the matrix to enhance the high-temperature strength of the alloy. In addition, Mo also contributes high-temperature strength through precipitation hardening. If the Mo content is less than 1.0%, its intended effects will not be attained. If the Mo content exceeds 3.5%, a deleterious phase will be precipitated to impair the ductility of the alloy. Hence, the Mo content of the Ni-base alloy of the present invention is specified to lie within the range of 1.0–3.5%, preferably 1.3–1.7%.

W: 3.5–4.5%

Tungsten is the same as Mo in that it has a dual capability for solid-solution hardening and precipitation hardening, contributing to the high-temperature strength of the alloy. To achieve its intended effects, W must be contained in an amount of at least 3.5%. If the W content is excessive, a deleterious phase will be precipitated and, at the same time, the specific gravity of the alloy will increase because tungsten itself is an element of high specific gravity and this is not only unfavorable for the purpose of using the alloy as a constituent material for fabricating the moving vanes of a turbine that will produce a centrifugal force upon rotation but also disadvantageous from an economic viewpoint. Hence, the W content of the Ni-base alloy of the present invention is specified to lie within the range of 3.5–4.5% preferably 4.1–4.5%.

Ta: 3.0–5.5%

Tantalum contributes to an improvement in the high-temperature strength of the alloy through solid-solution hardening and  $\gamma$  phase precipitation hardening. The effects of Ta will be exhibited if it is contained in an amount of at least 3.0%. If its addition is excessive, the ductility of the alloy will be impaired and, hence, the upper limit of the Ta content of the Ni-base alloy of the present invention is specified to be 5.5%, preferably 4.5–4.9%.

C: 0.06–0.12%

Carbon will form carbides that are precipitated preferentially at grain boundaries and dendrite boundaries to strengthen these boundaries, thereby contributing to an improvement in the high-temperature strength of the alloy.

To achieve its intended effects, carbon must be contained in an amount of at least 0.06%. However, if the C content exceeds 0.12%, the ductility of the alloy will be impaired. Hence, the C content of the Ni-base alloy of the present invention is specified to lie within the range of 0.06–0.12%.

B: 0.005–0.025%

Boron enhances the binding force at grain boundaries, thereby strengthening the matrix of the alloy to increase its high-temperature strength. To achieve its intended effects, boron must be contained in an amount of at least 0.005%. On the other hand, excessive addition of B can potentially impair the ductility of the alloy. Hence, the upper limit of the B content of the Ni-base alloy of the present invention is specified to be 0.025%.

Zr: 0.010–0.050%

Zirconium also enhances the binding force at grain boundaries, thereby strengthening the matrix of the alloy to increase its high-temperature strength. To achieve its intended effects, zirconium must be contained in an amount of at least 0.010%. On the other hand, excessive addition of Zr can potentially impair the ductility of the alloy. Hence, the upper limit of the Zr content of the Ni-base alloy of the present invention is specified to be 0.050%.

10 Mg and/or Ca: 1–100 ppm

Magnesium and/or calcium has a strong affinity with impurities such as oxygen and sulfur and they are also capable of preventing the decrease in ductility due to those impurities. If the content of Mg and/or Ca is less than 1 ppm, their intended effects will not be achieved. If, their content exceeds 100 ppm, the binding between grain boundaries will be attenuated rather than strengthened to eventually cause cracking. Hence, the content of Mg and/or Ca in the Ni-base alloy of the present invention is specified to lie within the range of 1–100 ppm.

15 Hf: 0–1.5%

Hafnium is capable of strengthening grain boundaries when columnar crystals are produced by unidirectional solidification. If hafnium is contained in an amount exceeding 1.5% it will bind with oxygen to form an oxide in the alloy, potentially causing cracks. Hence, the hafnium content of the Ni-base alloy of the present invention is specified to lie within the range of 0–1.5%.

20 At Least One Element of Pt, Rh and Re: 0–0.5%

These elements are effective in improving the corrosion resistance of the alloy. Even if their content exceeds 0.5%, no further improvement will be achieved. In addition, these elements are precious metals and using them in more than necessary amounts is not preferred from an economic viewpoint. Hence, the content of at least one of Pt, Rh and Re in the Ni-base alloy of the present invention is specified to lie within the range of 0–0.5%.

While the preferred ranges of the contents of Cr, Co, Mo, W, Ta, Al and Ti have been specified above with respect to the Ni-base heat-resistant alloy of the present invention, it should be noted that those elements will contribute to an improvement of the relative rupture life of the alloy if their combination and contents are properly selected.

The Ni-base heat-resistant alloy of the present invention 45 is described below in greater detail with reference to working examples.

## EXAMPLES

Nickel-base heat-resistant alloys having the compositions shown in Tables 1–3 were vacuum melted and the resulting melts were cast into a mold to make round bars having a diameter of 30 mm and a length of 150 mm. The bars were subjected to a solid-solution treatment by soaking at 1160° C. for 2 h and then to an aging treatment by soaking at 843° C. for 24 h, whereby samples of the Ni-base heat-resistant alloy of the present invention (Run Nos. 1–24), comparative samples (Run Nos. 1–4) and prior art samples (Run Nos. 1 and 2) were prepared. Prior art sample No. 1 was an equivalent of the alloy described in Japanese Patent Publication No. 59344/1989, supra and prior art sample Run No. 2 was an equivalent of commercially available Inconel (trademark) 738 as described in U.S. Pat. No. 3,459,545.

TABLE 1

| Element | Ni-base heat-resistant alloys of the invention |       |       |       |       |       |       |       |
|---------|------------------------------------------------|-------|-------|-------|-------|-------|-------|-------|
|         | 1                                              | 2     | 3     | 4     | 5     | 6     | 7     | 8     |
| Cr      | 13.1                                           | 14.0  | 15.0  | 13.5  | 14.5  | 13.3  | 14.2  | 13.8  |
| Co      | 9.0                                            | 8.5   | 10.1  | 10.5  | 9.7   | 8.8   | 9.3   | 9.5   |
| Mo      | 2.1                                            | 1.0   | 3.5   | 1.5   | 2.4   | 2.7   | 3.0   | 1.8   |
| W       | 4.0                                            | 3.5   | 4.3   | 3.7   | 4.5   | 4.1   | 3.9   | 4.2   |
| Ta      | 3.3                                            | 5.4   | 4.9   | 3.0   | 3.8   | 3.5   | 3.8   | 4.5   |
| Al      | 4.0                                            | 3.5   | 4.3   | 3.7   | 4.5   | 4.1   | 3.9   | 4.2   |
| Ti      | 2.7                                            | 2.3   | 3.2   | 2.5   | 2.9   | 3.0   | 2.8   | 2.7   |
| C       | 0.08                                           | 0.10  | 0.06  | 0.12  | 0.07  | 0.09  | 0.11  | 0.08  |
| B       | 0.011                                          | 0.009 | 0.007 | 0.015 | 0.013 | 0.012 | 0.010 | 0.005 |
| Zr      | 0.030                                          | 0.050 | 0.041 | 0.034 | 0.047 | 0.038 | 0.045 | 0.039 |
| Ca      | 54                                             | —     | 5     | 25    | 74    | 34    | 10    | 18    |
| Mg      | 22                                             | 98    | —     | 37    | 5     | 54    | 12    | 72    |
| Hf      | —                                              | —     | 1.1   | 0.7   | 1.2   | 0.9   | 0.8   | —     |
| Pt      | —                                              | —     | —     | —     | 0.5   | —     | —     | 0.05  |
| Rh      | —                                              | —     | —     | —     | —     | 0.3   | —     | —     |
| Re      | —                                              | —     | —     | —     | —     | —     | 0.4   | 0.05  |
| Ni      | bal.                                           | bal.  | bal.  | bal.  | bal.  | bal.  | bal.  | bal.  |

All numerals refer to percent by weight, except for Ca and Mg whose contents are indicated in ppm.

TABLE 2

| Element | Ni-base heat-resistant alloys of the invention |       |       |       |       |       |       |       |
|---------|------------------------------------------------|-------|-------|-------|-------|-------|-------|-------|
|         | 9                                              | 10    | 11    | 12    | 13    | 14    | 15    | 16    |
| Cr      | 13.1                                           | 14.0  | 15.0  | 13.5  | 14.5  | 13.3  | 14.2  | 13.8  |
| Co      | 9.0                                            | 8.5   | 10.1  | 10.5  | 9.7   | 8.8   | 9.3   | 9.5   |
| Mo      | 2.1                                            | 1.0   | 3.5   | 1.5   | 2.4   | 2.7   | 3.0   | 1.8   |
| W       | 4.0                                            | 3.5   | 4.3   | 3.7   | 4.5   | 4.1   | 3.9   | 4.2   |
| Ta      | 3.3                                            | 5.3   | 4.9   | 3.0   | 3.8   | 3.5   | 3.8   | 4.5   |
| Al      | 4.0                                            | 3.5   | 4.3   | 3.7   | 4.5   | 4.1   | 3.9   | 4.2   |
| Ti      | 2.7                                            | 2.3   | 3.2   | 2.5   | 2.9   | 3.0   | 2.8   | 2.7   |
| C       | 0.08                                           | 0.10  | 0.06  | 0.12  | 0.07  | 0.09  | 0.11  | 0.08  |
| B       | 0.011                                          | 0.009 | 0.007 | 0.015 | 0.013 | 0.012 | 0.010 | 0.005 |
| Zr      | 0.030                                          | 0.050 | 0.041 | 0.034 | 0.047 | 0.038 | 0.045 | 0.039 |
| Ca      | 54                                             | —     | 99    | 25    | 74    | 34    | 10    | 18    |
| Mg      | 22                                             | 98    | —     | 37    | 5     | 54    | 12    | 72    |
| Hf      | —                                              | —     | 1.5   | 0.7   | 1.2   | 0.9   | 0.8   | 1.3   |
| Pt      | 0.05                                           | 0.1   | —     | 0.2   | 0.06  | 0.2   | 0.05  | 0.08  |
| Rh      | 0.05                                           | 0.2   | 0.1   | 0.1   | —     | —     | 0.09  | —     |
| Re      | 0.05                                           | —     | 0.3   | —     | 0.07  | 0.1   | 0.05  | 0.2   |
| Ni      | bal.                                           | bal.  | bal.  | bal.  | bal.  | bal.  | bal.  | bal.  |
| Element | 17                                             | 18    | 19    | 20    | 21    | 22    | 23    | 24    |
| Cr      | 14.1                                           | 13.8  | 13.9  | 14.2  | 14.1  | 13.9  | 14.0  | 14.0  |
| Co      | 9.9                                            | 10.2  | 10.3  | 9.6   | 9.8   | 9.9   | 9.9   | 10.0  |
| Mo      | 1.5                                            | 1.6   | 1.6   | 1.4   | 1.4   | 1.5   | 1.5   | 1.5   |
| W       | 4.3                                            | 4.4   | 4.3   | 4.1   | 4.4   | 4.5   | 4.3   | 4.3   |
| Ta      | 4.6                                            | 4.8   | 4.8   | 4.6   | 4.7   | 4.6   | 4.7   | 4.7   |
| Al      | 4.1                                            | 4.1   | 4.0   | 3.9   | 3.9   | 4.1   | 4.0   | 4.0   |
| Ti      | 2.8                                            | 2.6   | 2.7   | 2.7   | 2.8   | 2.6   | 2.6   | 2.7   |
| C       | 0.08                                           | 0.09  | 0.08  | 0.10  | 0.07  | 0.06  | 0.09  | 0.09  |
| B       | 0.014                                          | 0.011 | 0.009 | 0.013 | 0.012 | 0.025 | 0.019 | 0.015 |
| Zr      | 0.037                                          | 0.022 | 0.013 | 0.023 | 0.021 | 0.039 | 0.030 | 0.02  |
| Ca      | —                                              | 12    | —     | 28    | 37    | 18    | 10    | —     |
| Mg      | 31                                             | 5     | 80    | 29    | 51    | 50    | 14    | 10    |
| Hf      | —                                              | —     | 0.3   | 0.2   | 0.2   | —     | 0.4   | —     |
| Pt      | —                                              | —     | —     | —     | 0.1   | —     | 0.02  | —     |
| Rh      | —                                              | —     | —     | —     | 0.1   | —     | 0.02  | —     |
| Re      | —                                              | —     | —     | —     | 0.1   | —     | 0.2   | —     |
| Ni      | bal.                                           | bal.  | bal.  | bal.  | bal.  | bal.  | bal.  | bal.  |

All numerals refer to percent by weight, except for Ca and Mg whose contents are indicated in ppm.

TABLE 3

| Element | Comparative Ni-base heat-resistant alloys |       |       |       | Prior art Ni-base heat-resistant alloys |       |
|---------|-------------------------------------------|-------|-------|-------|-----------------------------------------|-------|
|         | 1                                         | 2     | 3     | 4     | 1                                       | 2     |
| Cr      | *12.5                                     | *15.5 | 14.0  | 13.5  | 9.0                                     | 16.1  |
| Co      | 9.0                                       | 8.5   | 10.1  | 10.5  | 9.5                                     | 9.8   |
| Mo      | 2.1                                       | 1.0   | 3.5   | 1.5   | 1.8                                     | 1.9   |
| W       | 4.0                                       | 3.5   | 4.3   | 3.7   | 10.0                                    | 2.5   |
| Ta      | 3.3                                       | 5.3   | 4.9   | 3.0   | 1.5                                     | 1.2   |
| Al      | 4.0                                       | 3.5   | 4.3   | 3.7   | 5.5                                     | 4.0   |
| Ti      | 2.7                                       | 2.3   | 3.2   | 2.5   | 2.7                                     | 3.1   |
| C       | 0.08                                      | 0.10  | 0.06  | 0.12  | 0.08                                    | 0.19  |
| B       | 0.011                                     | 0.009 | 0.007 | 0.015 | 0.015                                   | 0.020 |
| Zr      | 0.030                                     | 0.050 | 0.041 | 0.034 | 0.05                                    | 0.100 |
| Ca      | 54                                        | —     | *105  | 25    | —                                       | —     |
| Mg      | 22                                        | 98    | —     | *110  | —                                       | —     |
| Nb      | —                                         | —     | —     | —     | 1.0                                     | 1.0   |
| Hf      | 1.1                                       | 0.5   | 1.5   | 0.7   | 1.3                                     | —     |
| Pt      | 0.05                                      | —     | —     | —     | —                                       | —     |
| Rh      | 0.05                                      | 0.5   | —     | 0.07  | —                                       | —     |
| Re      | —                                         | —     | 0.3   | —     | —                                       | —     |
| Ni      | bal.                                      | bal.  | bal.  | bal.  | bal.                                    | bal.  |

All numerals refer to percent by weight, except for Ca and Mg whose contents are indicated in ppm.

The values with an asterisk are outside the scope of the invention.

All samples of Ni-base heat-resistant alloy were subjected to a high-temperature corrosion resistance test and a high-temperature creep rupture strength test by the following procedures and the results of the respective tests are shown in Tables 3-5.

#### High-temperature corrosion resistance test

Each sample that was in the form of a round bar having a diameter of 30 mm and a length of 150 mm was worked into a test piece measuring 10 mm in diameter by 100 mm in length. The test piece was held for 1 h in the flame of natural gas at a temperature of ca. 1100° C. that contained hydrogen sulfide gas and subjected to 50 cycles of cooling each lasting for 30 min. After these treatments, the scale deposited on the surface of each test piece was removed and its weight loss was measured. The high-temperature corrosion resistance of the samples was evaluated in terms of the weight loss relative to the value for the test piece of prior art sample Run No. 1.

#### High-temperature creep rupture strength test

Each sample in a round bar form was worked into a test piece measuring 6 mm in diameter by 25 mm in length in the area bounded by parallel sides. All of the thus prepared test pieces were held in an air atmosphere at a temperature of 871° C. under a load of 35 kg/mm<sup>2</sup> and their life to rupture (in hours) was measured. The high-temperature creep rupture strength of the samples was evaluated in terms of the relative life to rupture, with the value for prior art sample Run No. 1 being taken as unity.

TABLE 4

| Run No.                                        | Relative weight loss | Relative rupture life |
|------------------------------------------------|----------------------|-----------------------|
| Ni-base heat-resistant alloys of the invention | 1                    | 0.58                  |
|                                                | 2                    | 0.51                  |
|                                                | 3                    | 0.41                  |
|                                                | 4                    | 0.54                  |
|                                                | 5                    | 0.42                  |

TABLE 4-continued

| Run No. | Relative weight loss | Relative rupture life |
|---------|----------------------|-----------------------|
| 6       | 0.40                 | 1.5                   |
| 7       | 0.40                 | 1.3                   |
| 8       | 0.45                 | 1.3                   |
| 9       | 0.42                 | 1.5                   |
| 10      | 0.43                 | 1.2                   |
| 11      | 0.38                 | 1.4                   |
| 12      | 0.44                 | 1.3                   |

TABLE 5

| Run No.                                        | Relative weight loss | Relative rupture life |
|------------------------------------------------|----------------------|-----------------------|
| Ni-base heat-resistant alloys of the invention | 13                   | 0.39                  |
|                                                | 14                   | 0.47                  |
|                                                | 15                   | 0.44                  |
|                                                | 16                   | 0.48                  |
|                                                | 17                   | 0.41                  |
|                                                | 18                   | 0.43                  |
|                                                | 19                   | 0.40                  |
|                                                | 20                   | 0.43                  |
|                                                | 21                   | 0.35                  |
|                                                | 22                   | 0.40                  |
|                                                | 23                   | 0.38                  |
|                                                | 24                   | 0.43                  |
| Comparative Ni-base heat-resistant alloys      | 1                    | 1.08                  |
|                                                | 2                    | 0.14                  |
|                                                | 3                    | 0.14                  |
|                                                | 4                    | 0.48                  |
| Prior art Ni-base heat-resistant alloys        | 1                    | 1                     |
|                                                | 2                    | 0.54                  |

As one can see from the data shown in Tables 1-5, the alloy compositions of the present invention which had the Cr content adjusted to the range of 13.1-15.0% with W, Mo, Al, Ti, Ta, C, B, Zr and other elements being added in such amounts as to attain the best possible balance and which further contained Mg and/or Ca in a total amount of 1-100 ppm, in the optional presence of Hf and/or at least one of Pt, Rh and Re exhibited high corrosion resistance and creep rupture strength at elevated temperatures.

It can therefore be concluded that the Ni-base alloy of the present invention which is improved not only in high-temperature strength but also in resistance to oxidation and corrosion at elevated temperatures is particularly useful as a constituent material for the moving and stationary vanes of a gas turbine that is to contact combustion gases that contain oxidizing materials, or for the moving vanes of a hot blower, or for other machine parts that are to be exposed to elevated temperatures.

What is claimed is:

- In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.1-15.0% Cr, 8.5-10.5% Co, 1.0-3.5% Mo, 3.5-4.5% W, 3.0-5.5% Ta, 3.5-4.5% Al, 2.2-3.2% Ti, 0.06-0.12% C, 0.005-0.025% B, 0.010-0.05% Zr, 1-100 ppm of Mg and/or Ca, 0-1.5% Hf and 0-0.5% of at least one element selected from the group consisting of Pt, Rh and Re, with the remainder being Ni and incidental impurities, all percentages being on a weight basis, wherein said Ta contributes to an improvement in the high temperature strength of the nickel alloy through  $\gamma$  phase precipitation.

2. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.1–15.0% Cr, 8.5–10.5% Co, 1.0–3.5% Mo, 3.5–4.5% W, 3.0–5.5% Ta, 3.5–4.5% Al, 2.2–3.2% Ti, 0.06–0.12% C, 0.005–0.025% B, 0.010–0.05% Zr, 1–100 ppm of Mg and/or Ca, with the remainder being Ni and incidental impurities, all percentages being on a weight basis, wherein said Ta contributes to an improvement in the high temperature strength of the nickel alloy through  $\gamma$  phase precipitation.

3. The rotating blade or stationary vane of a gas turbine according to claim 2, wherein the nickel alloy is selected from the group consisting of

- (a) 13.1 weight % Cr, 9.0 weight % Co, 2.1 weight % Mo, 4.0 weight % W, 3.3 weight % Ta, 4.0 weight % Al, 2.7 weight % Ti, 0.08 weight % C, 0.011 weight % B, 0.030 weight % Zr, 54 ppm Ca, 22 ppm Mg and the balance being Ni;
- (b) 14.0 weight % Cr, 8.5 weight % Co, 1.0 weight % Mo, 3.5 weight % W, 5.4 weight % Ta, 3.5 weight % Al 2.3 weight % Ti, 0.10 weight % C, 0.009 weight % B, 0.050 weight % Zr, 98 ppm Mg and the balance being Ni;
- (c) 14.1 weight % Cr, 9.9 weight % Co, 1.5 weight % Mo, 4.3 weight % W, 4.6 weight % Ta, 4.1 weight % Al, 2.8 weight % Ti, 0.08 weight % C, 0.014 weight % B, 0.037 weight % Zr, 31 ppm Mg and the balance being Ni;
- (d) 13.8 weight % Cr, 10.2 weight % Co, 1.6 weight % Mo, 4.4 weight % W, 4.8 weight % Ta, 4.1 weight % Al, 2.6 weight % Ti, 0.09 weight % C, 0.011 weight % B, 0.022 weight % Zr, 12 ppm Ca, 5 ppm Mg and the balance being Ni;
- (e) 13.9 weight % Cr, 9.9 weight % Co, 1.5 weight % Mo, 4.5 weight % W, 4.6 weight % Ta, 4.1 weight % Al, 2.6 weight % Ti, 0.06 weight % C, 0.025 weight % B, 0.034 weight % Zr, 18 ppm Ca, 50 ppm Mg and the balance being Ni; and
- (f) 14.0 weight % Cr, 10.0 weight % Co, 1.5 weight % Mo, 4.3 weight % W, 4.7 weight % Ta, 4.0 weight % Al, 2.7 weight % Ti, 0.09 weight % C, 0.015 weight % B, 0.02 weight % Zr, 10 ppm Mg and the balance being Ni.

4. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.1–15.0%, Cr, 8.5–10.5% Co, 1.0–3.5% Mo, 3.5–4.5% W, 3.0–5.5% Ta, 3.5–4.5% Al, 2.2–3.2% Ti, 0.06–0.12% C, 0.005–0.025% B, 0.010–0.05% Zr, 1–100 ppm of Mg and/or Ca and 0.5–1.5% Hf, with the remainder being Ni and incidental impurities, all percentages being on a weight basis, wherein said Ta contributes to an improvement in the high temperature strength of the nickel alloy through  $\gamma$  phase precipitation.

5. The rotating blade or stationary vane of a gas turbine according to claim 4, wherein the nickel alloy is selected from the group consisting of

- (a) 15.0 weight % Cr, 10.1 weight % Co, 3.5 weight % Mo, 4.3 weight % W, 4.9 weight % Ta, 4.3 weight % Al, 3.2 weight % Ti, 0.06 weight % C, 0.007 weight % B, 0.041 weight % Zr, 5 ppm Ca, 1.1 weight % Hf and the balance being Ni;

(b) 13.5 weight % Cr, 10.5 weight % Co, 1.5 weight % Mo, 3.7 weight % W, 3.0 weight % Ta, 3.7 weight % Al, 2.5 weight % Ti, 0.12 weight % C, 0.015 weight % B, 0.034 weight % Zr, 25 ppm Ca, 37 ppm Mg, 0.7 weight % Hf and the balance being Ni;

(c) 13.9 weight % Cr, 10.3 weight % Co, 1.6 weight % Mo, 4.3 weight % W, 4.8 weight % Ta, 4.0 weight % Al, 2.7 weight % Ti, 0.08 weight % C, 0.009 weight % B, 0.013 weight % Zr, 80 ppm Mg, 0.3 weight % Hf and the balance being Ni; and

(d) 14.2 weight % Cr, 9.6 weight % Co, 1.4 weight % Mo, 4.1 weight % W, 4.6 weight % Ta, 3.9 weight % Al, 2.7 weight % Ti, 0.10 weight % C, 0.013 weight % B, 0.023 weight % Zr, 28 ppm Ca, 29 ppm Mg, 0.2 weight % Hf and the balance being Ni.

6. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.1–15.0% Cr, 8.5–10.5% Co, 1.0–3.5% Mo, 3.5–4.5% W, 3.0–5.5% Ta, 3.5–4.5% Al, 2.2–3.2% Ti, 0.06–0.12% C, 0.005–0.025% B, 0.010–0.05% Zr, 1–100 ppm of Mg and/or Ca and 0–0.5% of at least one element selected from the group consisting of Pt, Rh and Re, with the remainder being Ni and incidental impurities, all percentages being on a weight basis, wherein said Ta contributes to an improvement in the high temperature strength of the nickel alloy through  $\gamma$  phase precipitation.

7. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.1–15.0% Cr, 8.5–10.5% Co, 1.0–3.5% Mo, 3.5–4.5% W, 3.0–5.5% Ta, 3.5–4.5% Al, 2.2–3.2% Ti, 0.06–0.12% C, 0.005–0.025% B, 0.010–0.05% Zr, 1–100 ppm of Mg and/or Ca, 0.5–1.5% Hf and 0.05–0.5% of at least one element selected from the group consisting of Pt, Rh and Re, with the remainder being Ni and incidental impurities, all percentages being on a weight basis, wherein said Ta contributes to an improvement in the high temperature strength of the nickel alloy through  $\gamma$  phase precipitation.

8. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.7–14.3% Cr, 9.5–10.5% Co, 1.3–1.7% Mo, 4.1–4.5% W, 4.5–4.9% Ta, 3.8–4.2% Al, 2.5–2.9% Ti, 0.06–0.12% C, 0.005–0.025% B, 0.010–0.05% Zr and 1–100 ppm of Mg and/or Ca, with the remainder being Ni and incidental impurities, all percentages being on a weight basis, wherein said Ta contributes to an improvement in the high temperature strength of the nickel alloy through  $\gamma$  phase precipitation.

9. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.7–14.3% Cr, 9.5–10.5% Co, 1.3–1.7% Mo, 4.1–4.5% W, 4.5–4.9% Ta, 3.8–4.2% Al, 2.5–2.9% Ti, 0.06–0.12% C, 0.005–0.025% B, 0.010–0.05% Zr, 1–100 ppm of Mg and/or Ca, 0.1–1.5% Hf and 0–0.5% of at least one element selected from the group consisting of Pt, Rh and Re, with the remainder being Ni and incidental impurities, all percent-

60  
65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
6610  
6611  
6612  
6613  
6614  
6615  
6616  
6617  
6618  
6619  
6620  
6621  
6622  
6623  
6624  
6625  
6626  
6627  
6628  
6629  
6630  
6631  
6632  
6633  
6634  
6635  
6636  
6637  
6638  
6639  
6640  
6641  
6642  
6643  
6644  
6645  
6646  
6647  
6648  
6649  
66410  
66411  
66412  
66413  
66414  
66415  
66416  
66417  
66418  
66419  
66420  
66421  
66422  
66423  
66424  
66425  
66426  
66427  
66428  
66429  
66430  
66431  
66432  
66433  
66434  
66435  
66436  
66437  
66438  
66439  
66440  
66441  
66442  
66443  
66444  
66445  
66446  
66447  
66448  
66449  
66450  
66451  
66452  
66453  
66454  
66455  
66456  
66457  
66458  
66459  
66460  
66461  
66462  
66463  
66464  
66465  
66466  
66467  
66468  
66469  
66470  
66471  
66472  
66473  
66474  
66475  
66476  
66477  
66478  
66479  
66480  
66481  
66482  
66483  
66484  
66485  
66486  
66487  
66488  
66489  
66490  
66491  
66492  
66493  
66494  
66495  
66496  
66497  
66498  
66499  
664100  
664101  
664102  
664103  
664104  
664105  
664106  
664107  
664108  
664109  
664110  
664111  
664112  
664113  
664114  
664115  
664116  
664117  
664118  
664119  
664120  
664121  
664122  
664123  
664124  
664125  
664126  
664127  
664128  
664129  
664130  
664131  
664132  
664133  
664134  
664135  
664136  
664137  
664138  
664139  
664140  
664141  
664142  
664143  
664144  
664145  
664146  
664147  
664148  
664149  
664150  
664151  
664152  
664153  
664154  
664155  
664156  
664157  
664158  
664159  
664160  
664161  
664162  
664163  
664164  
664165  
664166  
664167  
664168  
664169  
664170  
664171  
664172  
664173  
664174  
664175  
664176  
664177  
664178  
664179  
664180  
664181  
664182  
664183  
664184  
664185  
664186  
664187  
664188  
664189  
664190  
664191  
664192  
664193  
664194  
664195  
664196  
664197  
664198  
664199  
664200  
664201  
664202  
664203  
664204  
664205  
664206  
664207  
664208  
664209  
664210  
664211  
664212  
664213  
664214  
664215  
664216  
664217  
664218  
664219  
664220  
664221  
664222  
664223  
664224  
664225  
664226  
664227  
664228  
664229  
664230  
664231  
664232  
664233  
664234  
664235  
664236  
664237  
664238  
664239  
664240  
664241  
664242  
664243  
664244  
664245  
664246  
664247  
664248  
664249  
664250  
664251  
664252  
664253  
664254  
664255  
664256  
664257  
664258  
664259  
664260  
664261  
664262  
664263  
664264  
664265  
664266  
664267  
664268  
664269  
664270  
664271  
664272  
664273  
664274  
664275  
664276  
664277  
664278  
664279  
664280  
664281  
664282  
664283  
664284  
664285  
664286  
664287  
664288  
664289  
664290  
664291  
664292  
664293  
664294  
664295  
664296  
664297  
664298  
664299  
664300  
664301  
664302  
664303  
664304  
664305  
664306  
664307  
664308  
664309  
664310  
664311  
664312  
664313  
664314  
664315  
664316  
664317  
664318  
664319  
664320  
664321  
664322  
664323  
664324  
664325  
664326  
664327  
664328  
664329  
664330  
664331  
664332  
664333  
664334  
664335  
664336  
664337  
664338  
664339  
664340  
664341  
664342  
664343  
664344  
664345  
664346  
664347  
664348  
664349  
664350  
664351  
664352  
664353  
664354  
664355  
664356  
664357  
664358  
664359  
664360  
664361  
664362  
664363  
664364  
664365  
664366  
664367  
664368  
664369  
664370  
664371  
664372  
664373  
664374  
664375  
664376  
664377  
664378  
664379  
664380  
664381  
664382  
664383  
664384  
664385  
664386  
664387  
664388  
664389  
664390  
664391  
664392  
664393  
664394  
664395  
664396  
664397  
664398  
664399  
664400  
664401  
664402  
664403  
664404  
664405  
664406  
664407  
664408  
664409  
664410  
664411  
664412  
664413  
664414  
664415  
664416  
664417  
664418  
664419  
664420  
664421  
664422  
664423  
664424  
664425  
664426  
664427  
664428  
664429  
664430  
664431  
664432  
664433  
664434  
664435  
664436  
664437  
664438  
664439  
664440  
664441  
664442  
664443  
664444  
664445  
664446  
664447  
664448  
664449  
664450  
664451  
664452  
664453  
664454  
664455  
664456  
664457  
664458  
664459  
664460  
664461  
664462  
664463  
664464  
664465  
664466  
664467  
664468  
664469  
664470  
664471  
664472  
664473  
664474  
664475  
664476  
664477  
664478  
664479  
664480  
664481  
664482  
664483  
664484  
664485  
664486  
664487  
664488  
664489  
664490  
664491  
664492  
664493  
664494  
664495  
664496  
664497  
664498  
664499  
664500  
664501  
664502  
664503  
664504  
664505  
664506  
664507  
664508  
664509  
664510  
664511  
664512  
664513  
664514  
664515  
664516  
664517  
664518  
664519  
664520  
664521  
664522  
664523  
664524  
664525  
664526  
664527  
664528  
664529  
664530  
664531  
664532  
664533  
664534  
664535  
664536  
664537  
664538  
664539  
664540  
664541  
664542  
664543  
664544  
664545  
664546  
664547  
664548  
664549  
664550  
664551  
664552  
664553  
664554  
664555  
664556  
664557  
664558  
664559  
664560  
664561  
664562  
664563  
664564  
664565  
664566  
664567  
664568  
664569  
664570  
664571  
664572  
664573  
664574  
664575  
664576  
664577  
664578  
664579  
664580  
664581  
664582  
664583  
664584  
664585  
664586  
664587  
664588  
664589  
664590  
664591  
664592  
664593  
664594  
664595  
664596  
664597  
664598  
664599  
664600  
664601  
664602  
664603  
664604  
664605  
664606  
664607  
664608  
664609  
664610  
664611  
664612  
664613  
664614  
664615  
664616  
664617  
664618  
664619  
664620  
664621  
664622  
664623  
664624  
664625  
664626  
664627  
664628  
664629  
664630  
664631  
664632  
664633  
664634  
664635  
664636  
664637  
664638  
664639  
66

ages being on a weight basis, wherein said Ta contributes to an improvement in the high temperature strength of the nickel alloy through  $\gamma$  phase precipitation.

10. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 14.0% Cr, 10.0% Co, 1.5% Mo, 4.3% W, 4.7% Ta, 4.0% Al, 2.7% Ti, 0.09% C, 0.015% B, 0.02% Zr and 10 ppm of Mg, with the remainder being Ni and incidental impurities, all percentages being on a weight basis, wherein said Ta contributes to an improvement in the high temperature strength of the nickel alloy through  $\gamma$  phase precipitation.

11. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.1–15.0% Cr, 9.5–10.5% Co, 1.0–3.5% Mo, 3.5–4.5% W, 3.0–5.5% Ta, 3.5–4.5% Al, 2.2–3.2% Ti, 0.06–0.12% C, 0.005–0.025% B, 0.010–0.05% Zr, 1–100 ppm of Mg and/or Ca, 0.05–0.5% Rh, with the remainder being Ni and incidental impurities, all percentages being on a weight basis, wherein said Ta contributes to an improvement in the high temperature strength of the nickel alloy through  $\gamma$  phase precipitation.

12. In a rotating blade or stationary vane of a gas turbine, wherein the improvement comprises the rotating blade or stationary vane being made of a nickel alloy that has high strength and high resistance to oxidation and corrosion at elevated temperatures and that consists essentially of 13.1–15.0% Cr, 8.5–10.5% Co, 1.0–3.5% Mo, 3.5–4.5% W, 3.0–5.5% Ta, 3.5–4.5% Al, 2.5–3.2% Ti, 0.06–0.12% C, 0.005–0.025% B, 0.010–0.05% Zr, 1–100 ppm of Mg and/or Ca, 0.5–1.5% Hf and 0.05–0.5% of Rh, with the remainder being Ni and incidental impurities, all percentages being on

a weight basis, wherein said Ta contributes to an improvement in the high strength of the nickel alloy through  $\gamma$  phase precipitation.

13. In a rotating stationary vane of a gas turbine, wherein the improvement comprises the rotating blade or stationary vane being made of a nickel alloy that has high strength and high resistance to oxidation and corrosion at elevated temperatures and that consists essentially of 13.7–14.3% Cr, 9.5–10.5% Co, 1.3–1.7% Mo, 4.1–4.5% W, 4.5–4.9% Ta, 3.8–4.2% Al, 2.5–2.9% Ti, 0.06–0.12% C, 0.005–0.025% B, 0.010–0.05% Zr, 1–100 ppm of Mg and/or Ca, 0–1.5% Hf and 0–0.5% of at least one element selected from the group consisting of Pt, Rh and Re, with the remainder being Ni and incidental impurities, all percentages being on a weight basis, wherein said Ta contributes to an improvement in the high strength of the nickel alloy through  $\gamma$  phase precipitation.

14. The rotating blade or stationary vane of a gas turbine according to claim 13, wherein said Hf is in an amount of 0.5–1.5% and said at least one element selected from the group consisting of Pt, Rh and Re is in an amount of 0.05–0.5%.

15. In a rotating blade or stationary vane of a gas turbine, wherein the improvement comprises the rotating blade or stationary vane being made of a nickel alloy that has high strength and high resistance to oxidation and corrosion at elevated temperatures and that consists of 13.1–15.0% Cr, 8.5–10.5% Co, 1.0–3.5% Mo, 3.5–4.5% W, 3.0–5.5% Ta, 3.5–4.5% Al, 2.2–3.2% Ti, 0.06–0.12% C, 0.005–0.025% B, 0.010–0.05% Zr, 1–100 ppm of Mg and/or Ca, 0–1.5% Hf and 0.05–0.2% of Re, with the remainder being Ni and incidental impurities, all percentages being on a weight basis, wherein said Ta contributes to an improvement in the high temperature strength of the nickel alloy through  $\gamma$  phase precipitation.

\* \* \* \* \*